

Oct. 16, 1945.

A. L. FEILD

2,387,130

ALLOY PROCESS

Filed Jan. 31, 1941

*FIG. 1.*



*FIG. 2.*



INVENTOR

Alexander L. Feild  
John Howard Joynt  
HIS ATTORNEY

## UNITED STATES PATENT OFFICE

2,387,130

## ALLOY PROCESS

Alexander L. Feild, Towson, Md., assignor to  
Rustless Iron and Steel Corporation, a corpora-  
tion of Delaware

Application January 31, 1941, Serial No. 376,918

3 Claims. (Cl. 75—130.5)

My invention relates to the production of an iron-chromium-silicon alloy of low carbon content which is useful as a pre-alloy in the production of stainless steel.

Among the objects of my invention are the production of an iron-chromium-silicon pre-alloy of high chromium and silicon contents, in combination with a low carbon content, in a simple, efficient, economical and thoroughly practical manner, employing available melting and furnacing equipment, and using inexpensive and available, semi-prepared materials or raw materials such as ores, including low grade chrome ore when desired, permitting a wide flexibility between the choice of semi-prepared materials, in solid or molten forms, and yielding a high grade product, with maximum metal per unit of melting equipment, and all with a minimum consumption of power and labor, and full economy of continuous operation.

Other objects, in part will be obvious and in part pointed out hereinafter.

The invention accordingly consists in the several operational steps, and the relation of each of the same to one or more of the others as described herein, the useful application of which is indicated in the claims.

In the accompanying drawing, illustrating certain features of my invention:

Fig. 1 is a flow sheet for the production of ferro-chrome-silicon according to one aspect of my invention; and

Fig. 2 is a flow sheet of a modified method of producing ferro-chrome-silicon according to another aspect of the invention.

As conducive to a clearer understanding of certain features of my invention, it may be noted at this point that ferrochrome silicon is finding use as an inexpensive source of chromium in the production of stainless steel. This is particularly true where it also serves as a reducing agent. See for example the process of producing stainless steel described in the U. S. Letters Patent 1,954,381 issued to me on April 10, 1934, and entitled Manufacture of rustless iron. Attention also is directed to the process of my co-pending application for U. S. Letters Patent Serial No. 372,400 filed December 30, 1940, and entitled Production of stainless steel.

Ferrochrome-silicon, according to heretofore used practices, commonly is produced by smelting together chrome ore, quartzite and coke. An electric arc furnace of the submerged electrode type ordinarily is employed. I find, however, that this process is not feasible commercially where the

chrome ore available is of a low grade. The slag volume becomes excessive, the power consumption prohibitive and the production rate so low as to make the process wholly impractical.

Accordingly an object of the present invention is the provision of a simple, efficient and practical process for the production of ferrochrome-silicon, using available and inexpensive low grade chrome ore, using known and available furnacing equipment, all with minimum power consumption and without encountering unmanageable volumes of slag.

Referring now more particularly to the practice of my invention, attention is directed to Fig. 1 of the drawing. In manufacturing an iron-chromium-silicon pre-alloy in accordance with my invention I melt together quantities of a chromium-iron pre-alloy and a ferro-silicon. In accordance with certain features of my invention, I produce a high carbon, chromium-iron pre-alloy by smelting together quantities of chrome ore and a carbonaceous reducing agent such as coke in a ferro-alloy furnace. Secondly I produce ferro-silicon, by smelting together quantities of a carbonaceous reducing agent such as coke and a high silica raw material such as crushed quartzite in a second ferro-alloy furnace. Desired quantities of the two melts are combined in a steel making furnace of the Heroult type.

After the ferrochrome and ferrosilicon are prepared as above, I charge them into the Heroult steel making furnace in such quantities that the ratio of available silicon to chromium contents of the charge ranges between approximately  $\frac{1}{2}$  to 1 and 2 to 1. Carbon is expelled from the mixture during the steel furnacing stage, this carbon rising to the surface of the melt. The carbon on the surface of the melt oxidizes or combines with the slag so that it can be subsequently skimmed off. After skimming off the slag, I tap the furnace withdrawing molten low carbon ferrochrome-silicon pre-alloy. The final product is cooled and retained in desired form for future use in the manufacture of stainless steel.

In order that my invention may be more clearly understood, it may be noted at this point that the great thirst of a chromium steel bath for carbon is well recognized in the metallurgy art. A chromium-containing steel bath also has a thirst for silicon. Where, however, carbon and silicon both are present in the bath I have discovered that silicon, when present in sufficient amounts, will cause carbon to be expelled freely from the bath. The explanation for this feature may be that once there is sufficient silicon in the chro-

mium-iron bath to combine with the chromium, carbon will not be permitted to do so. Thus, the carbon is expelled from the bath. I do not, however, wish to be bound by this explanation.

I find that the ratio of silicon to chromium, necessary to expel carbon and give the desired low carbon ferrochrome-silicon pre-alloy, ranges between substantially  $\frac{1}{2}$  to 1 and 2 to 1. Silicon as noted above, for some reason not fully known to me, causes carbon to be expelled from the bath of metal. Further, the amount of carbon expelled increases, and the amount remaining in the melt decreases, as the ratio of silicon to chromium in the melt is increased. Thus, in order to obtain the desired low carbon ferrochrome-silicon pre-alloy, it is essential that the ferrosilicon employed contain sufficient silicon to displace the carbon of the ferrochrome. Accordingly, where a high grade chrome ore is employed in making the high carbon ferrochrome pre-alloy, the silicon content of the ferrosilicon ingredient, with which the ferrochrome pre-alloy is combined, preferably should be high. In ferro-chrome pre-alloys made from low grade chrome ore, the chromium present of course, will not be so great. Consequently, the silicon content of the ferrosilicon may be lower, although it will be understood that the quantity of ferrosilicon necessary may be decreased where the higher silicon material is used.

As a specific example of the practice of my invention, I conveniently use a three-phase ferro-alloy furnace, rated 6000 k. v. a. in producing the ferrochrome. Preferably the furnace is lined with magnesite. Ferrosilicon conveniently is prepared in a like ferro-alloy furnace, this preferably being lined with carbon brick. Finally, I prepare the low carbon ferrochrome-silicon pre-alloy, preferably by combining the ferrochrome pre-alloy and ferrosilicon in a three-phase Heroult electric-arc furnace rated 3500 k. v. a. To minimize lining attack, this furnace preferably is lined with silica brick, backed up with magnesite. I do not wish, however, to limit my invention to the use of any particular type of furnace, furnace lining or other appurtenant structure in any one of the operations disclosed herein, since it will be readily understood by those skilled in the art that considerable latitude of choice exists in the selection of means to be used in carrying out my invention.

It is to be observed that in the practice of my invention, the chrome ore charged into the first of the above mentioned pre-alloy furnaces well may be of a low grade. In fact my process, as distinguished from conventional processes, is adapted to use such an ore, without encountering the unmanageable slag volumes ordinarily met with. The grade of this ore may be so low as to contain only some 25% to 40% chromic oxide ( $\text{Cr}_2\text{O}_3$ ). The ferrochrome pre-alloy yield usually analyzes 35% to 75% chromium, with a carbon content of 4% to 8% or more and the remainder principally iron.

The ferrosilicon obtained from the second pre-alloy furnace, previously mentioned, ordinarily contains a large amount of silicon while the remainder thereof is principally iron. Usually a ferro-silicon containing at least 40% silicon is required for, as stated above, silicon is largely responsible for the expulsion of carbon from the final ferro-chrome-silicon heat. I prefer to use ferrosilicon containing at least 65% silicon.

In my process, the relative quantities of high carbon ferro-chrome and ferro-silicon used are

such as to produce directly a ferrochrome-silicon pre-alloy with a maximum carbon content of 0.2%, approximately 30% to 60% chromium, 60% to 28% silicon and the remainder principally iron.

The relative proportions of the desirable constituents, iron, chromium and silicon; and the elimination of carbon in my ferrochrome-silicon pre-alloy can, for example, be controlled by analysis of the raw ingredients available for the preparation of ferrochrome pre-alloy and ferrosilicon, or by separate analysis of the ferrochrome pre-alloy and the ferrosilicon before they are combined, or by analysis of a test heat which contains ferrochrome pre-alloy and ferrosilicon in predetermined proportions. Such trial and error methods when practiced by the metallurgist soon enables him to predict with reasonable certainty, the content of the final ferrochrome-silicon product and also to know the proper amounts of ferrochrome pre-alloy and ferrosilicon needed in the melt to produce desired results.

Another somewhat modified method of practicing my invention is illustrated in Fig. 2 of the drawing. Here, as in the method previously described, I prepare a high carbon, ferrochrome pre-alloy by smelting together quantities of low grade chrome ore and coke in a ferro-alloy furnace of the type previously mentioned. In a second ferro-alloy furnace, of the type formerly described, I smelt together quantities of coke and crushed quartzite or other silica product. During the smelting operations in the two furnaces, molten ferrochrome pre-alloy is tapped in regulated amounts from the first furnace and is fed over the charge in the second furnace. As a result the ferrochrome pre-alloy combines with the ferrosilicon as it is produced in the second furnace. Carbon is expelled from the combined melts in the second furnace and apparently is oxidized in the slag.

As before, I proportion the amounts of ferrochrome employed and the quartzite and coke so as to regulate the chromium, iron, silicon and carbon contents of the resultant ferrochrome-silicon. Also the grades of raw materials and the quality of the ferrochrome and ferrosilicon are similar to those specified above.

Accordingly, it will be seen that my invention provides for the production of a low carbon ferrochrome-silicon pre-alloy, in which the silicon and chromium contents are high, using available and inexpensive low grade chrome ores. This is to be distinguished from the conventional, expensive practice of smelting chrome ore, silica and coke to give a ferrochrome-silicon pre-alloy of low carbon content, which practice is not commercially feasible where low grade chrome ores are employed because of the excess slag volumes encountered as noted above.

While in practicing my invention, I preferably mix selected proportions of molten ferrochrome pre-alloy and molten ferrosilicon in the final heat, I find it expedient under certain circumstances to incorporate one of the ingredients in solid form with the other in molten form or to heat together desired proportionate parts of solid ferrochrome and solid ferrosilicon. Such modified practices at times are more satisfactory than the practice of combining the ingredients strictly in molten form. These modifications in the methods of carrying out my invention are made so as to have full economy of continuous operation of the ferro-alloy furnaces with a minimum consumption of power and labor. Any excess ferrochrome or ferrosilicon is tapped off and per-

mitted to solidify and cool after which it is stored for future use.

While certain types of raw materials are designated, and while certain proportions of iron, chromium, silicon and carbon are described as being preferable in the materials which I use and in the finished product, it is to be understood that these materials and the proportions thereof are illustrative only.

As many possible embodiments may be made of my invention, and as many changes may be made in the embodiments hereinbefore set forth, it is to be understood that all matter described herein, or shown in the accompanying drawing, is to be interpreted as illustrative and not as a limitation.

I claim:

1. In the production of an iron-chromium-silicon pre-alloy comprising approximately 30% to 60% chromium, 60% to 28% silicon, with a maximum carbon content of .20% and the remainder principally iron, the art which includes smelting crushed quartzite and coke with an iron-chromium pre-alloy separately prepared by smelting a low grade chrome ore containing 25% to 40% chromic oxide and comprising 35% to 75% chromium with a carbon content of 4% to 8% and the remainder iron, the ingredients being in such quantity that the ratio of the available silicon to chromium contents of the charge ranges between approximately  $\frac{1}{2}$  to 1 and 2 to 1 whereby carbon is expelled from the melt, and thereafter removing the carbon from the surface of the melt and tapping the melt free of carbon.

2. In the production of an iron-chromium-sili-

con pre-alloy of low carbon content, the art which includes, smelting chrome ore containing 25% to 40% chromic oxide with coke in a first furnace giving a melt containing at least 35% chromium and substantial amounts of carbon, smelting quartzite with coke in a second furnace, charging the melt from the first furnace into the second furnace before or during the smelting operation in such proportions that the available silicon-to-chromium ratio ranges between approximately one-half to one and two to one whereby carbon is expelled from the resultant combined melt, and thereafter tapping the melt substantially free of carbon.

3. In the production of an iron-chromium-silicon pre-alloy comprising approximately about 30% to 60% chromium, 60% to 28% silicon with a maximum carbon content of .20% and the remainder principally iron, the art which includes smelting chrome ore containing from about 25% to 40% chromic oxide with a carbonaceous reducing agent and giving an iron-chromium pre-alloy comprising about 35% to 75% chromium and the remainder iron and carbon; separately smelting crushed quartzite and a carbonaceous reducing agent; charging into the smelting furnace before or during the smelting operation said iron-chromium prealloy in such quantity that the ratio of the available silicon to chromium contents of the charge ranges between approximately  $\frac{1}{2}$  to 1 and 2 to 1, whereby carbon is expelled from the melt; and tapping the melt substantially free of carbon.

ALEXANDER L. FEILD.